

Patented June 2, 1925.

1,540,354

# UNITED STATES PATENT OFFICE.

FRANK C. MATHERS, OF BLOOMINGTON, INDIANA.

## ELECTROLYTE FOR ELECTROPLATING METAL WITH TIN.

No Drawing.

Application filed March 29, 1923. Serial No. 628,433.

To all whom it may concern:

Be it known that I, FRANK C. MATHERS, a citizen of the United States, residing at Bloomington, county of Monroe, State of

5 Indiana, have invented a certain new and useful Improvement in Electrolyte for Electroplating Metal with Tin, of which the following is a full, clear, and exact description.

10 My invention relates to the electroplating of sheets of metal or other metallic objects with tin and has for its object to deposit electrolytically a dense, thick coating of finely crystalline structure, free from projections and of a substantially uniform thickness.

15 A further object of my invention is to provide a process in which a thick coating of such a character can be produced at a rapid rate and in a relatively short time.

20 By thick coating I mean a coating of a thickness equal to, or over, one thousandth (.001) of an inch.

25 In a patent granted to me on November 15, 1921, No. 1,397,222, I have described a process of electrolytic refining of tin, in which the anode was composed of a mixture of tin and lead and in which the electrolyte used contained hydrofluosilicic acid, or its equivalent, together with sulphuric acid and 30 a small amount of cresylic acid and glue. In carrying out that process the current was passed from the anode to the cathode, resulting in the dissolving of the anode and the depositing of the tin from the solution of the 35 electrolyte upon the cathode, the lead combining with the sulphuric acid and adhering to the anode as an insoluble substance. The deposit made upon the cathode by the process of that patent with its three-tenths per 40 cent (0.3%) of cresylic acid, except when such deposit is formed slowly by the use of a comparatively small current, is in the form of a coarse, crystalline, solid deposit of substantially uniform thickness, having a rough 45 and an ununiform surface but strongly coherent. Such a deposit is all that is necessary for refining purposes.

50 I have discovered that cresylic acid when used in a tin plating bath, under proper conditions, enables me to attain results which have long been desired and sought for without success. When added to a tin sulphate bath, for instance, or to the bath described in U. S. Patent No. 916,155 granted 55 to H. L. Hollis, March 23, 1909, it enables me to obtain a much thicker coating than

has heretofore been practicable, and to obtain such a coating in a time which renders thick electroplating commercial and valuable.

60 In carrying out my present invention, in its preferred form, I use anodes composed of commercially pure tin, and an electrolyte composed of an acid solution of sulphate of tin, preferably about 20° Baumé which corresponds to a specific gravity 1.158, to which I add cresylic acid, the amount of cresylic acid being such as to make a substantially saturated solution. I also preferably add about .7% by weight of animal glue.

65 The density of the tin sulphate can be varied through wide limits and still give good deposits. The rate of deposit should be decreased, however, as the density is lessened. It is important, however, in order to 70 obtain the highest grade deposit to maintain the cresylic acid near the saturation point. For a fair deposit at a slower rate, half saturation by cresylic acid is permissible.

75 As is well known, free acid must be present in an aqueous solution of tin sulphate or other tin salts in order to prevent hydrolysis, which would take place if the solution were neutral. This condition is preferably obtained by using an excess of sulphuric acid. 80 The cresylic acid in my electroplating process functions as an addition agent to prevent the formation of coarsely crystalline cathode deposits, and not to prevent hydrolysis. Cresylic acid is not, properly 85 speaking, an acid and does not practically prevent hydrolysis, if at all.

90 The tin salt I use comprises tin in the stannous condition combined with at least one, by which I mean one or more, of the acid forming elements of series 2 and 3 of Mendeleef's Periodic Table and included in Groups III, IV, VI and VII thereof, and having atomic weights of less than 33, the preferred salt being tin sulphate. Mendeleef's Table is to be found on pages 50 and 95 51 of "A Treatise on Chemistry" by Roseoe and Schlorlemmer, Vol. 2, published by Macmillan & Co., 1913.

100 The object to be plated is placed in the bath so as to form a cathode and the plating current applied. A current of about 16 amperes per square foot of surface at a voltage of 1½ volts secures proper results, although with a higher voltage and more current the 110 time for electroplating may be reduced. The object while within the bath is preferably

kept in motion to detach hydrogen bubbles or foreign substances suspended in the bath, the motion, when a sheet is being plated, being in the plane of the sheet. Annealed 5 sheets, on account of the smoothness of coating, can be finished by so few passes through the rolls that they will still be soft. If hard copper is desired, the sheets may be rolled so as to harden them either before or after 10 plating.

In the case of continuous lengths of strips or wire, the continuous lengths are passed slowly through an elongated bath, proper 15 electrical connections being maintained, every portion being kept within the bath for a period corresponding to the thickness desired.

My process, while particularly useful in 20 the production of tin coated copper, can be used for coating sheets or fabricated articles of iron or steel or other metals or alloys.

The electrolyte when once formed is a 25 practically stable electrolyte except for the cresylic acid and glue which are gradually consumed during the electroplating process and must be replaced from time to time as required.

The expression "cresylic acid" as used 30 herein is used broadly to mean the more complex oily phenol-like bodies which are somewhat soluble in water. I preferably use the cresylic acid, known as cresol, in its crude commercial form.

With the current and voltage and the electrolyte above referred to, a coating of a 35 thickness of two thousandths (.002) of an inch can be obtained in about an hour and other thicknesses in proportionate periods. The coating thus formed is smooth, uniformly dense, of a fine crystalline structure, 40 free from projections and of substantially uniform thickness. If a sheet thus coated is passed through rolls a few times it can be easily buffed so as to take a very high polish.

45 If finished sheets of comparatively soft

copper are desired, the sheets when placed in the bath should be in an annealed or soft condition.

As will be evident to those skilled in the art my invention permits of various modifications without departing from the spirit thereof or the scope of the appended claims. 50

What I claim is:

1. An electrolyte for electroplating with 55 tin composed essentially of a solution of tin sulphate and cresylic acid sufficient in quantity to cause an electrolyte deposit of tin from the solution to be finely crystalline and smooth.

2. An electrolyte for electroplating with 60 tin comprising an acid plating solution of a soluble tin salt comprising tin in stannous condition combined with at least one acid forming element of series 2 and 3 of Mendeleef's Periodic Table and included in 65 Groups III, IV, VI and VII thereof, and having an atomic weight of less than 33, approximately saturated with cresylic acid.

3. An electrolyte for electroplating with 70 tin composed essentially of a solution of tin sulphate approximately saturated with cresylic acid.

4. An electrolyte for electroplating with 75 tin comprising an acid plating solution of a soluble tin salt of approximately 20° Baume comprising tin in stannous condition combined with at least one acid forming element of series 2 and 3 of Mendeleef's Periodic Table and included in Groups III, IV, VI and VII thereof, and having an atomic 80 weight of less than 33, and cresylic acid.

5. An electrolyte as characterized in claim 1, with the addition of glue.

6. An electrolyte as characterized in claim 2 with the addition of glue.

7. An electrolyte as characterized in claim 3 with the addition of glue.

8. An electrolyte as characterized in claim 4 with the addition of glue.

FRANK C. MATHERS.